

July 2, 1929.

A. R. LUKENS ET AL

1,719,118

ASPHALT SURFACED ROOFING

Filed Dec. 29, 1922



Fig. 1.



Fig. 2.

INVENTOR  
A. R. Lukens  
Joseph S. Magnan  
By *Acme* *Allen*  
ATTORNEYS

Patented July 2, 1929.

1,719,118

# UNITED STATES PATENT OFFICE.

ALAN R. LUKENS, OF WYOMING, AND JOSEPH S. MAYNARD, OF CINCINNATI, OHIO,  
ASSIGNORS, BY MESNE ASSIGNMENTS, TO THE FLINTKOTE COMPANY, OF BOSTON,  
MASSACHUSETTS, A CORPORATION OF MASSACHUSETTS.

## ASPHALT-SURFACED ROOFING.

Application filed December 29, 1922. Serial No. 609,749.

Our invention relates to the surfacing of roofs, and more particularly to the adequate and inexpensive protection of so-called built-up roofs having a layer of asphalt uppermost.

5 In the construction of built-up roofs layers of fibrous material, such as felt composition, are placed on the roof structure, and then molten asphalt or tar is poured onto the felt, and further layers of felt and asphalt or tar 10 are applied, with the roof being finished with a layer of the molten bitumen, which is covered with crushed slag or clean screened gravel. In the case of asphalt it has not always been customary to employ any mineral 15 dressing. A tar of sufficient hardness not to slip is very shiny, and will check, crumble and crack unless thickly covered with a dressing, of gravel or slag, usually weighing 400 pounds to the square of 100 square feet of 20 roof.

It is known that the surface of asphalt when exposed to the rays of light of the sun is affected actinically, so as to become "cheesy" and liable to promote further disintegration. 25 While this fact was known to the chemist, it has not been considered of importance in protecting the asphalt coating of roofs, or if it has been recognized, it has been disregarded, and the builders have contented 30 themselves with the observation that asphalt-surfaced roofs have proved satisfactory, theory to the contrary notwithstanding.

In the preparation of prepared roofing it has been the practice to surface it with 35 crushed slate, which is rolled into the surface, and in the so-called rubber roofing it has been the practice to apply a lubricant in the form of talc or mica to prevent sticking. Also, as above noted, it has been the practice to provide a hard surface of pebbles or 40 slag for built-up roofs.

It may be observed that in each of the cases noted there has in fact been applied a coating or dressing of material which to varying extent, cuts off light from access to the asphalt 45 itself.

In view of the fact, however, that this protection to the asphalt from actinic disintegration has been unconscious, the various methods for covering the asphalt in built-up and prepared roofings have been either ineffective or expensive from the point of view of application.

It is the object of our invention to provide,

as a result of our discoveries, a top dressing 55 for asphalt or other bituminous roofings of opaque finely divided mineral matter having great surface area as compared to weight, and thus to protect against actinic rays with the maximum efficiency and at the least expense.

It is not our object primarily to apply these protective coatings in the factory onto prepared roofing, since the best form of protective material will be black, insoluble, dull 65 in surface, and very permanent in the weather.

Such a material, so far as we have been able to select one, is always of a hard abrasive quality, and thus would be too dangerous to 70 workmen, who would breathe it in, to permit of its use in a closed factory building.

With suitable protection to the workman it could be used, however, and would give a very effective and well appearing "rubber" 75 roofing product.

The use of slag or pebbles does not fully protect asphalt or tar poured in a layer on the top of a roof structure, unless it is quite thick, and even then light can get through 80 the cracks between the pebbles. Slag is perhaps better than pebbles in this respect. But in either case the material is quite heavy, and has a high cost of transportation, and is expensive to use on the building, due to transportation and application difficulties.

Talc or mica used on an asphalt roof, while effective to a partial degree in protecting against actinic rays, would not serve as sufficient protection, in our opinion, were it not 90 for the fact that soot and dust of more opaque quality are also deposited on the roof. Both talc and mica are of translucent quality.

We prefer to use a light powder composed of a dull black colored substance. The dullness makes the substance light absorbing, so that it does not reflect light. The act of reflection often serves to permit a considerable quantity of light to penetrate through a thin film of the substance, which is not desired.

The substance must also be insoluble, and very permanent against corrosion or disintegration, due to the effects of the weather.

We have found a substance in nature composed of a hydrated ferrous oxide combined 105 with silicon, which is amorphous in quality and is not known geologically as until our invention, herein described, it has had no com-

mercial use. It was called by the copper manufacturer which makes the material a by-product of copper production, a slag powder, and among many other powdered materials tried, it was the only one which in a very thin layer would not transmit actinic rays of light.

Referring to the drawings, Figure 1 represents a perspective view of a cut-away corner of a roof in the treatment of which our invention has been used. Figure 2 represents a cross section of the roof portion shown in Figure 1. The powdered mineral matter 1 is shown as spread over the hot bitumen 2 which is applied on and covers in a thin layer the roofing felt 3.

A few pounds of this substance scattered or (and) brushed onto a top layer of bitumen in a roof, when same is still hot, will serve to cover a normal layer of several hundred pounds of asphalt, and thus a top dressing or coating for built-up roofs may be provided, using a suitable asphalt, with which can be readily shipped small cans of the product that the workman can carry on his person. The powdery nature of the product insures a complete coverage without chance for seepage of light, this being more or less impractical with larger particles. The powder is applied while the roof is hot, so that it is held fast by the tacky bituminous coating.

The comparison in weight, cost of transportation and expense between the standard gravel or slag finishes for bituminous roofs are naturally very favorable to our top dressing.

Other substances of like characteristics may

be obtained and we have given the above as preferred because of its cost and physical properties, aside from its light protecting function.

Carboniferous material of lubricating quality we do not favor, because of the likelihood of its running, and thus creating a danger of staining the sides of a building.

Our experiments have indicated that a roof covered with a layer of plain asphalt with a dark colored non-reflective powder will completely withstand disintegration under the influence of light, and thus the roofs prepared according to our invention are just as good and much lighter in weight than gravel or slag covered roofs, and have an equal or longer life, since asphalt if not subjected to the breaking down effect of light is strongly resistant to acid, alkali, heat and cold, and electrolysis, and our coating material is easy to form into a continuous surface on the asphalt and hence our roofs are as permanent a covering as can be produced, if properly protected, and easier to produce in a perfect manner than any roofs of this type known to us.

Having thus described our invention, what we claim as new and desire to secure by Letters Patent, is:—

A roof comprising an upper surface of asphalt and a thin surfacing layer of hydrated ferrous oxide combined with silicon in powdery form, said thin layer being sufficient to cut off substantially all actinic light rays from access to the asphalt.

ALAN R. LUKENS.  
JOSEPH S. MAYNARD.